

No. 806,047.

PATENTED NOV. 28, 1905.

R. BAGGALY.

METHOD OF SMELTING AND CONVERTING ORES.

APPLICATION FILED OCT. 11, 1904. RENEWED OCT. 13, 1905.



WITNESSES

Warren W. Gwarty  
L. A. Conner

INVENTOR

Ralph Baggaley

# UNITED STATES PATENT OFFICE.

RALPH BAGGALY, OF PITTSBURG, PENNSYLVANIA.

## METHOD OF SMELTING AND CONVERTING ORES.

No. 806,047.

Specification of Letters Patent.

Patented Nov. 28, 1905.

Application filed October 11, 1904. Renewed October 13, 1905. Serial No. 282,677.

*To all whom it may concern:*

Be it known that I, RALPH BAGGALY, of Pittsburgh, Allegheny county, Pennsylvania, have invented a new and useful Method of 5 Smelting and Converting Ores, of which the following is a full, clear, and exact description, reference being had to the accompanying drawing, forming part of this specification, which shows in vertical cross-section a 10 converter suitable for the practice of my invention.

The object of my invention is to smelt and convert ores, particularly copper, gold, and silver bearing ores, in a manner which is an 15 improvement upon the process described in Patent No. 766,654, issued to Ralph Baggaley and Charles M. Allen on August 2, 1904.

In the patent just referred to the preferred procedure consisted in melting a primary bath 20 of low-grade sulfid ores to the extent of approximately the holding capacity of the converter and thereafter feeding into such molten bath silicious mineral-bearing raw ores in relatively small proportions to the volume 25 of such molten bath—that is to say, in amount less than the volume of such molten bath—in order that the raw ores might be dissolved partly by the heat of the molten bath and partly by the intense heat produced by the 30 oxidizable elements and compounds contained in the molten bath through the action of the air-blast.

My present invention is practiced, preferably, by the following method of procedure:

(A.) The use of a larger converting vessel 35 than at present used, or, in other words, preferably one capable of holding ten, thirty, or even fifty tons of ore or molten matte or slag at one time. Such vessel is shown at 2 in the 40 drawing.

(B.) Such vessel preferably to be made of heavy metal blocks in order that the heat produced by the process shall be absorbed and conserved by such blocks instead of being 45 rapidly carried away and wasted, as must be the case where water-jackets of any kind are utilized.

(C.) The placing within this converter of a relatively large proportion of raw mineral-bearing ores—say in a total of thirty tons of ore under treatment twenty-five or twenty-seven tons to be in the raw state.

(D.) The cementing of this body 3 of raw

ore into position opposite the twyers 4, as shown in the drawing, by means of a layer of 55 molten matte or slag.

(E.) Placing thereafter into such converter a relatively small proportion of sulfid ores high in fuel values—say in a total of thirty tons of ore under treatment three tons or five 60 tons to be thus placed in the converter in the molten state or sufficient to cover the converting-twyers and to provide the requisite liquid matte with which through the action of the converting blast intense heat may be generated, whereby the twenty-seven tons of raw ore may thus be quickly melted down practically without the use of carbonaceous fuel, and such mineral-bearing raw ores thereafter to constitute a part of the molten bath in the 70 converter. After all of the raw ores have thus been melted down practically without carbonaceous fuel in the manner described the converting process is thereafter continued in the usual way until the molten bath is 75 thereby reduced to blister-copper and poured from the converter into molds.

After the raw ore has been reduced to the molten condition as described other ores in the raw state may be from time to time added 80 at will and dissolved by the heat of the molten bath or of the converting process. Such additions of raw ore will thereafter be dissolved and constitute a part of the molten bath. In this manner the process may be almost indefinitely continued, at least up the point where the holding capacity of the converter in white metal (i. e., seventy-six per cent. matte) has been reached, or the heat of the molten bath may be augmented at will by the simple addition of ores in the raw state that are relatively high in fuel values. Should an excess 85 of iron exist in the molten bath, this may be readily fluxed by the addition of ores whose distinctive feature is high in silica, or, indeed, 90 by the addition of practically pure silica without associated mineral values, if desired. In the same manner lime or other flux in the raw state may be added to the molten bath at will.

Through this method of treating ores their 100 mineral contents may readily be recovered without any of the losses incident to water concentration and to calcination and practically without the use of carbonaceous fuel, since in treating, say, a total of thirty tons 105 of ore carbonaceous fuel would only be utilized.

ized in melting the first three tons with which the process is started, and then after the twenty-seven tons of raw ore had thus been melted almost indefinite additions of raw ore may be 5 added in continuing the melting process entirely without the use of carbonaceous fuel.

The heavy consumption of coke or other carbonaceous fuel in smelting copper ores is usually not due to the mere fusion of the ore 10 proper. It is due to the fact that calcination and consequently the enrichment of the ore before actual fusion is forced to the utmost limit within the blast-furnace. The mere melting of sulfid ores in a blast-furnace without 15 any attempt at calcination or enrichment may easily be accomplished through the combustion of from one to two per cent. of carbonaceous fuel, providing an adequate smelting blast is provided.

20 In practicing this art it is my desire to avoid enrichment of the sulfid ore during the operation of melting it, because any enrichment necessarily reduces the fuel elements contained in the sulfid ores after fusion, which it 25 is my desire to utilize thereafter in effective work in melting raw mineral-bearing ores in the converter.

Doubtless many variations or modifications 30 in the details of this process will suggest themselves to those skilled in the art without

departing from the spirit of my invention, since

What I claim is—

1. The method of smelting and converting ores, which consists in placing in a vessel a 35 relatively large mass of raw ore, and adding a relatively small proportion of molten matte high in fuel values, and subjecting the matte to an air-blast; substantially as described.

2. The method of smelting and converting 40 ores, which consists in placing in a vessel a relatively large mass of raw ore, sealing it in position, and adding a relatively small proportion of molten matte high in fuel values, and subjecting the matte to an air-blast; sub- 45 substantially as described.

3. The method of smelting and converting ores, which consists in placing in a vessel a 50 relatively large mass of raw ore, sealing it in position opposite to the twyers and adding a relatively small proportion of molten matte high in fuel values, and subjecting the matte to an air-blast; substantially as described.

In testimony whereof I have hereunto set my hand.

RALPH BAGGALY.

Witnesses:

H. M. CORWIN,  
JOHN MILLER.